# EUROPEAN PATENT APPLICATION

(11) **EP 3 693 479 A1**
(43) Date of publication of application: **12.08.2020**
(21) Application number: 20155854.1
(22) Date of filing: 06.02.2020
(51) Int. Cl.: C21D 1/00, C21D 1/20, C21D 1/25, C21D 1/607, C21D 8/02

(54) **METHOD FOR PRODUCING AUSFERRITIC STEEL AND DUCTILE IRON, AUSTEMPERED IN RAPID CYCLES FOLLOWED BY BAKING**

(30) Priority: 08.02.2019 SE 1950152
(71) Applicant: Ausferritic AB, 922 21 Vindeln (SE)
(72) Inventor: LARKER, Richard, 922 32 Vindeln (SE)
(74) Representative: Valea AB

(57) **Abstract**

Method for producing an ausferritic steel or an ausferritic ductile iron, which comprises the steps of subjecting a steel alloy having a silicon content of 1.5-4.4 wt% Si and a carbon content of 0.3-0.8 wt% C, or a ductile iron having a silicon content of 2.0-4.6 wt% Si and a carbon content of 2.9-3.8 wt% C, to an austempering heat treatment comprising the following steps: austenitizing said steel alloy or ductile iron, quenching said steel alloy or ductile iron at a cooling rate that is sufficiently high to prevent predominant formation of proeutectoid ferrite or pearlite, transforming austenite in said quenched steel alloy or ductile iron into an ausferritic structure, and subsequently baking said steel alloy or ductile iron at one or more temperatures to complete said transformation of any remaining austenite into ausferrite, to equalize the carbon distribution within its austenite phase, and to temper any martensite that has formed, to produce an ausferritic steel or an ausferritic ductile iron having a microstructure containing at least 50 volume-% of ausferrite with superior properties at a substantially lower process cost.

## Description

### TECHNICAL FIELD

The present invention concerns a method for producing ausferritic steel and ductile iron austempered in rapid cycles followed by baking in air at low temperature in an oven, said ausferritic steel and ductile iron being suitable for cost-efficient production of components requiring high or very high strength and high or very high ductility and/or fracture toughness, wherein the silicon content prevents bainite formation and promote a predominantly ausferritic (which for steels has also been described as "carbide-free bainitic", "nanobainitic" or "superbainitic" in the prior art) microstructure during austempering also when formation is accomplished close above the initial Mₛ temperature, and increases the solid solution strengthening by silicon and carbon of the resulting acicular ferrite.

### BACKGROUND OF THE INVENTION

In a typical austempering heat treatment cycle, work pieces comprising steel or ductile cast iron with graphite spheroids are firstly heated and then held at an austenitizing temperature in a furnace until they become austenitic and the carbon from dissolved prior cementite in pearlite is evenly distributed in the austenite formed. In steel alloys the carbon content is fixed in prior production steps, while in ductile irons the carbon content in the steel-like matrix between the dispersed graphite spheroids can be varied by the selection of the austenitization temperature during heat treatment, since the solubility of carbon in austenite increases with temperature and carbon can readily diffuse between matrix and graphite. In ductile irons, the austenite must therefore be given enough time to be saturated with carbon diffusing from the graphite, especially if the matrix is partly ferritic or fully ferritic at ambient temperature. Together with the more complex solidification structure and segregation of alloying elements in ductile irons vs. steels, the soak time necessary for austenitization is usually longer for ductile irons than for steels, typically between 1.0-2.5 hours (longer when alloyed for hardenability in larger cross-sections) while 0.5-1.5 hours may be sufficient for steels. In both cases the soak time may be reduced by using a higher austenitization temperature, since the carbon diffusivity increases rapidly with temperature.

After the work pieces are austenitized, they are quenched (usually in a salt bath) at a quenching rate that is high enough to avoid the formation of pearlite or proeutectoid ferrite during quenching down to an intermediate temperature below the pearlite region in the continuous cooling transformation (CCT) diagram but above the initial Mₛ temperature, at which the austenite having this level of carbon would otherwise start to transform into martensite.

This austempering range of intermediate temperatures is better known as the bainitic range for common low-silicon steels.

The work pieces are then held for a time sufficient for a usually isothermal transformation to ausferrite at this temperature denoted the "austempering" temperature (which can be confusing since the complete heat treatment process is also denoted "austempering"), after which they are allowed to cool to ambient temperature.

In a similar way to the bainitic structures formed by similar heat treatments of low-silicon steels, final microstructure and properties of ausferritic materials are strongly influenced by the austempering temperature and holding time at that temperature. The ausferritic microstructure becomes coarser at higher transformation temperatures and finer at lower temperatures. In contrast to bainitic structures formed in low-silicon steels, nucleation and growth of acicular or feathery ferrite (depending on formation temperature) are generally not accompanied by formation of bainitic carbides, since this is delayed or prevented by the higher silicon content. Instead, the partial diffusion of carbon leaving the ferrite formed enriches the surrounding austenite, stabilizing the austenite with carbon by reducing its Mₛ far below ambient temperature.

The resulting duplex matrix microstructure is denoted "ausferrite" (although it can in steels also be denoted "nanobainite", "superbainite" or "carbide-free bainite"), consisting of acicular or feathery ferrite being nucleated and grown within concurrently carbon stabilized austenite.

At higher isothermal transformation temperatures, the coarser and mainly feathery ferrite is nucleated and grown in a matrix of relatively thick films of carbon stabilized austenite with a larger relative amount of austenite (which may promote higher ductility if the austenite is sufficiently stabilized with carbon), while at lower isothermal transformation temperatures, the increasingly fine and increasingly acicular ferrite is nucleated and grown in a matrix of relatively thin films of carbon stabilized austenite with a larger relative amount of ferrite (enabling higher strength).

A lower isothermal transformation temperature improves the nucleation rate of ferrite due to larger undercooling of the austenite, while a higher isothermal transformation temperature increases the carbon diffusivity and thus improves both the growth rate of the ferrite and the increased and equalized carbon content in the stabilized austenite. Since this transformation from austenite to ferrite is governed by carbon diffusion under para-equilibrium conditions (although the opinion is still predominant that this transformation is diffusion-less in carbide-free bainitic steels), the transformation is initially rapid when diffusion distances are short but gradually slows down when the change in microstructure is close to completion, while the equalization of the carbon distribution within the austenite phase to increase its mechanical stability may take even longer time. Similar to the influence on the prior austenitization step, the more complex solidification structure and segregation of alloying elements in ductile irons vs. steels usually require longer soak durations in the "austempering" step for ductile irons than for steels, typically between 1.5-4.0 hours (longer when alloyed for hardenability in larger cross-sections) while 0.75-1.5 hours may be sufficient for steels. The "process window" may also be limited at excessively long soak durations when the high-carbon austenite desired for the mechanical properties may decompose to ferrite plus bainitic carbides, but an increased silicon content delays this decomposition process to unpractically longer soak durations.

Austempered ductile iron (ADI) (which has previously incorrectly been referred to as "bainitic ductile iron" even though when correctly heat treated, ADI contains no bainite) represents a special family of ductile (spheroidal graphite) cast iron alloys which possess improved strength and ductility properties. Compared to as-cast ductile irons, ADI castings are at least twice as strong at the same ductility level, or show at least twice the ductility at the same strength level.

In most cast irons including ductile irons, silicon levels of at least two weight percent in the ternary Fe-C-Si system are necessary to promote grey solidification resulting in graphite inclusions. When austempered, the increased silicon level further delays or completely prevents the formation of embrittling bainite (ferrite + cementite Fe₃C) during austempering, as long as the austempering temperature is relatively far above the Mₛ temperature and the austempering time is not too prolonged.

This freedom of bainitic carbides in "upper ausferrite" results in ductile properties (while in low-silicon steels "upper bainite" obtained at similar temperatures is brittle due to the location of its carbides). When austempering of conventional ductile irons is performed at low temperatures, their silicon contents of about 2.3-2.7 wt% Si are not sufficient to completely prevent the formation of bainitic carbides in "lower ausferrite". Such microstructures contain fine acicular ferrite as their major phase, thin carbon stabilized austenite as well as some bainitic carbide, resulting in considerable decrease in ductility, fatigue strength and machinability.

Recently, as-cast ductile iron grades with silicon contents higher than 3 wt% Si have been standardized, where their matrices are completely ferritic with increasing solid solution strengthening of the ferrite, providing concurrently increased yield strength and ductility compared to conventional ferritic-pearlitic ductile irons of the same ultimate tensile strength levels (450-600 MPa).

Such solution strengthened ductile irons have recently been used as precursors for austempering in development of the SiSSADI™ (**S**ilicon **S**olution **S**trengthened **ADI**) concept by the present inventor. In order to obtain complete austenitization, higher temperatures are necessary (since the austenite field in the phase diagram shrinks with increasing silicon); otherwise any remaining proeutectoid ferrite both reduces the hardenability during quench (since nucleation of pearlite in austenite only is slow but growth of pearlite on any remaining proeutectoid ferrite is rapid) and reduces the resulting mechanical properties (since less ausferrite can be formed).

Benefits from increased silicon include shorter time both during austenitization (since carbon diffusion increases rapidly with increasing temperature) and during austempering (since silicon promotes the precipitation of ferrite), increased solution strengthening of the acicular ferrite (by both silicon and carbon), freedom of bainitic carbides also in "lower ausferrite" formed close above initial Mₛ, and as a result concurrently improved strength and ductility.

Ausferritic steels can be obtained by similar heat treatments as for ausferritic irons, on condition that the steels contain sufficient silicon to reduce or prevent the precipitation of bainitic carbides. An example of rolled commercial steels that are suitable for austempering to form ausferrite (without or with low contents of bainitic carbides) instead of bainite is the spring steel EN 1.5026 with a typical composition containing 0.55 wt% C, 1.8 wt% Si and 0.8 wt% Mn.

When steels with sufficiently high silicon contents are austempered, they have usually been described as "carbide-free bainite", "nanobainite" or "superbainite", implying that the major part of the carbon leaving the formed ferrite is enriching and stabilizing the surrounding austenite instead of forming bainitic carbides.

International publication WO 2016/022054 by the present inventor describes austempered steel from the development of the SiSSASteel™ (**S**ilicon **S**olution **S**trengthened **A**usferritic **Steel**) concept for components requiring high strength and high ductility and/or fracture toughness, which has a silicon content of 3.1-4.4 wt% Si and a carbon content of 0.4-0.6 wt% C and a microstructure that is ausferritic. A method for producing such an austempered steel is also disclosed.

The method comprises the step of conducting an austempering heat treatment including complete austenitization, whereby the higher the silicon content of the steel, the higher the austenitization temperature.

For example, the austempered steel may be produced by forming a melt comprising steel with a silicon content of 3.1-4.4 wt% Si and a carbon content of 0.4-0.6 wt% C, casting from the melt a component or a semi-finished bar, allowing the component or semi-finished bar to be forged or rolled before cooling or to cool directly, optionally followed by forging and subsequent cooling, then heat treating the cooled component, semi-finished bar or forging at a first temperature and holding the component, semi-finished bar or forging at the temperature for a predetermined time to completely austenitize the component, semi-finished bar or forging, quenching the heat treated component, semi-finished bar or forging at a quenching rate sufficient to prevent the formation of pearlite during quenching down to an intermediate temperature below the pearlite region in the continuous cooling transformation (CCT) diagram but above the Mₛ temperature, such as a quenching rate of at least 150 °C/min, heat treating the component, semi-finished bar or forging at one or several temperatures above the Mₛ temperature for a predetermined time to austem-per said component, semi-finished bar or forging, resulting in an ausferritic steel.

### SUMMARY OF THE INVENTION

An object of the present invention is to provide an improved method for cost efficient production of ausferritic steel and ausferritic ductile iron (ADI) with improved mechanical properties that are produced by subjecting a steel alloy or a ductile iron respectively to a rapid austempering heat treatment as compared to conventional austempering heat treatments. The steel alloy or ductile iron is austenitized, quenched and transformed into a predominantly ausferritic structure (usually isothermally in a salt bath although any suitable quenching medium may be used and/or the transformation need not necessarily be isothermal), followed by baking in an oven in a suitable atmosphere, such as in air at one or more temperatures to finish the transformation into a predominantly ausferritic structure with equalized carbon distribution within its austenite phase, thereby improving the mechanical properties of the ausferritic steel and ausferritic ductile iron, especially the 0.2% proof strength and the elongation at fracture.

This object is achieved by a method for producing ausferritic materials, namely an ausferritic steel or an ausferritic ductile iron, which comprises the steps of subjecting a steel alloy having a silicon content of 1.5-4.4 wt% Si and a carbon content of 0.3-0.8 wt% C or a ductile iron having a silicon content of 2.0-4.6 wt% Si and a carbon content of 2.9-3.8 wt% C (mainly as spheroidal graphite) to an austempering heat treatment followed by baking. After austenitization, the cooling rate during quenching is sufficiently high to prevent predominant formation of proeutectoid ferrite or pearlite, while the subsequent transformation of the under-cooled austenite to predominantly ausferrite may either take place at one or more temperatures above the Mₛ temperature of the austenite having initial carbon content (before quench), or initially by cooling to a lower temperature to form some martensite whereupon the acicular ferrite can efficiently nucleate and grow at a usually higher temperature. When baking is adopted as a process step after the austempering heat treatment, the transformation into ausferrite may only need to proceed until all austenite volumes (both the film-like austenite between ferrite sheaves and the blocky austenite) have been enriched sufficiently with carbon to depress their Mₛ temperature below ambient, thereby limiting the amount of martensite being formed when cooled to ambient temperature or lower.

The subsequent baking, in air in an oven for example, is able to continue and complete the transformation of carbon enriched austenite into ausferrite, with improved mechanical stability of the austenite phase by equalization of its carbon content, and to temper any martensite previously formed (where tempering embrittlement in the intermediate temperature range is prevented by the silicon content), the method resulting in cost efficient production of ausferritic steel and ductile iron with improved mechanical properties and having a predominantly ausferritic microstructure.

According to an embodiment of the invention the ausferritic steel or the ausferritic ductile iron matrix has a microstructure that contains less than 10 vol% of proeutectoid ferrite.

According to an embodiment of the invention the ausferritic steel or the ausferritic ductile iron matrix has a microstructure that contains less than 40 vol% of tempered martensite, or less than 30 vol% of tempered martensite, or less than 20 vol% of tempered martensite or less than 10 vol% of tempered martensite.

According to an embodiment of the invention the ausferritic steel or ausferritic ductile iron is suitable for components requiring high strength and high ductility and/or fracture toughness. According to an embodiment of the invention the austempered steel has a silicon content of 3.1-4.4 wt% Si and a carbon content of 0.4-0.6 wt% C.

According to an embodiment of the invention the austempered ductile iron has a silicon content of 2.0-4.6 wt% Si and a carbon content of 2.9-3.8 wt% C (mainly as spheroidal graphite).

The method namely comprises the steps of subjecting a steel alloy having a silicon content of 1.5-4.4 wt% Si and a carbon content of 0.3-0.8 wt% C or subjecting a ductile iron having a silicon content of 2.0-4.6 wt% Si and a carbon content of 2.9-3.8 wt% C (mainly as spheroidal graphite) to an austempering heat treatment followed by baking, where austenite areas not yet transformed to ausferrite, but having carbon contents intermediate between the initial medium carbon austenite after the austenitizing step and the films of austenite stabilized by high carbon content in ausferritic areas, will transform to new ausferritic areas having a microstructure with fineness and ferrite-austenite proportions similar to ausferrite formed isothermally at the same temperature after quench. Concurrently any martensite formed earlier will be tempered and contribute to the strength of the ausferritic steel or ausferritic ductile iron.

This method results in the cost efficient production of austempered steel or austempered ductile iron having an ausferritic microstructure, i.e. the microstructures are predominantly, if not completely, ausferritic. A predominantly ausferritic microstructure is intended to mean that the steel or the ductile iron matrix contains at least 50 vol% of ausferrite, at least 60 vol% of ausferrite, at least 70 vol% of ausferrite, at least 80 vol% of ausferrite, and typically at least 90 vol% of ausferrite.

The microstructure may also, if the hardenability of the alloy is insufficient for the cooling rate above the austempering temperature range, contain a small amount (2-8vol%) of proeutectoid ferrite and even lower amounts of pearlite, since the high Si content delays cementite formation.

In addition, the microstructure may contain some martensite if the cooling is deliberately continued below the initial Mₛ temperature during quench or austempered for a shorter time than necessary for all austenite volumes to have their Mₛ temperatures decreased below ambient temperature, but such thermally induced martensite will subsequently be tempered during the baking process step.

It should be noted that the produced ausferritic steel or ductile iron components do not necessarily need to be cooled to ambient temperature before baking is started, but baking may start while the components are still at a temperature above the ambient temperature, thereby limiting or completely preventing any formation of martensite. There is also an option to increase the formation of martensite if the steel is cooled to temperatures lower than ambient temperature before baking, in order to increase the contribution to strength from martensite tempered during the baking in an oven.

The term "oven" as used in this document may be any device used for heating at least one part of one or more workpieces or maintaining at least one part of one or more workpieces at a particular temperature or within a particular temperature range, in air for example. Workpieces may be placed entirely or partly within an oven and treated either batch wise or continuously in a belt oven. Alternatively, an "oven" may comprise one or more heating means placed adjacently to, along, or around one or more workpieces in order to heat at least one part of the one or more workpieces to a particular temperature or to maintain at least one part of the one or more workpieces at a particular temperature or within a particular temperature range.

If the time in the austempering temperature range after quenching is too short for the austenite to transform completely into ausferrite, the remaining austenite areas will either transform to thermally induced martensite during cooling to ambient temperature making the steel brittle, or when mechanically loaded decrease properties by firstly causing an early plastic deformation in any incompletely transformed austenite areas with lower carbon content resulting in reduced yield strength, and secondly fracture early with reduced ultimate tensile strength at reduced elongation when the deforming austenite transforms too soon at by far too low strains into mechanically induced brittle martensite.

These limitations in mechanical properties can be eliminated by cost-effective baking in a suitable atmosphere, such as in air, at one or more temperatures within the austempering temperature range, in far less costly equipment per process hour than the integrated salt bath furnaces that have conventionally been used for austempering heat treatments, where the soak time in salt bath is generally longer than the prior soak time in the austenitization furnace, and therefore the soak time in the salt bath limits the productivity. During baking, in air for example, in the austempering temperature range the austenite areas having intermediate carbon content will continue to transform into ausferritic microstructures, being in fineness and ferrite-austenite proportions similar to ausferrite formed isothermally at same temperature after quench during conventional austempering. Concurrently the diffusion of carbon continues, enriching and equalizing the carbon distribution in the austenite phase, thereby increasing its mechanical stability. The resulting microstructure may therefore consist of more than one ausferritic morphologies, one formed during the usually isothermal transformation in salt bath after quench, the other with morphology governed by temperature vs. time during the cost efficient baking process step in air, being either isothermal or not (such as heating and cooling zones at the ends if a belt oven).

The invention is based on the finding that it is possible to concurrently improve mechanical properties of ausferritic materials and substantially reduce costs for austempering heat treatments by increasing the productivity in integrated salt bath furnaces through shortened soak time in salt bath, when combined with subsequent inexpensive baking in air to complete the transformation into mechanically stable ausferrite, resulting in a more robust process providing superior and less varying mechanical properties.

Surprisingly, it was found that the conversion into predominantly ausferrite was firstly sufficiently achieved during a shortened soak time in salt bath as compared with conventional austempering heat treatments, and then completed during baking in air for example despite high alloying contents for hardenability (Cr + Ni + Mo + V in steel, Ni + Cu + Mo in ductile iron), which a skilled person would have expected to delay the conversion.

According to an embodiment of the invention the ausferritic steel or the ausferritic ductile iron matrix has a microstructure that is substantially carbide-free or that contains very small volume fractions of carbides, i.e. less than 1 vol% of carbides.

According to an embodiment of the invention the ausferritic steel has the following composition in weight percent:

| | |
|---|---|
| C | 0.3-0.8 |
| Si | 1.5-4.4 |
| Mn | max 4.0 |
| Cr | max 25.0 |
| Cu | max 2.0 |
| Ni | max 20.0 |
| Al | max 2.0 |
| Mo | max 6.0 |
| V | max 0.5 |
| Nb | max 0.2 |

balance Fe and normally occurring impurities. P and S are preferably kept to a minimum.

According to an embodiment of the invention the ausferritic ductile iron has the following composition in weight percent:

| | |
|---|---|
| C | 2.9-3.8 |
| Si | 2.0-4.6 |
| Mn | max 0.4 |
| Cu | max 1.2 |
| Ni | max 2.0 |
| Mo | max 0.3 |

balance Fe and normally occurring impurities. P and S are preferably kept to a minimum.

The method according to the present invention is namely suitable for the production of ausferritic steel or ausferritic ductile iron having any suitable chemical composition. Preferred compositions have high silicon contents, i.e. a silicon content of 3.1-4.4 wt% Si in ausferritic steel or 3.35-4.6 wt% Si in ausferritic ductile iron, irrespective of the amounts of the other alloying elements as long as the maximum values above are not exceeded.

According to an embodiment of the invention the preferred ausferritic steel has a silicon content of at least 1.6, 1.7, 1.8, 1.9, 2.0, 2.1, 2.2, 2.3, 2.4, 2.5, 2.6, 2.7, 2.8, 2.9, 3.0, 3.1, 3.2, 3.3, 3.4, 3.5, 3.6, 3.7, 3.8, 3.9 or 4.0 wt% Si and/or a carbon content of at least 0.4 or 0.5 wt% C.

Additionally or alternatively, the preferred ausferritic steel that has a maximum silicon content of 4.3, 4.2, 4.1, 4.0, 3.9, 3.8, 3.7, 3.6 or 3.5 wt% Si and/or a maximum carbon content of 0.6 or 0.5 wt% C.

According to an embodiment of the invention the preferred austempered ductile iron has a silicon content of at least 3.35, 3.4, 3.5, 3.6, 3.7, 3.8, 3.9, 4.0, 4.1 or 4.2 wt% Si.

Additionally or alternatively, the preferred austempered ductile iron hat has a maximum silicon content of 4.6, 4.5, 4.4, 4.3, 4.2, 4.1, 4.0, 3.9, 3.8 or 3.7 wt% Si.

The word "max" throughout this document is intended to mean that the ausferritic steel or ductile iron comprises from 0 wt% (i.e. including 0 wt%) up to and including the indicated maximum amount of the element in question. The produced ausferritic steel or ausferritic ductile iron may therefore comprise low levels of such elements when not needed for hardenability or other reasons, i.e. levels of 0-0.1 wt%. The produced ausferritic steel or ausferritic ductile iron may however comprise higher levels of at least one or any number of these elements for optimizing the process and/or final properties, i.e. levels including the indicated max amount or levels approaching the indicated max amount to within 0.1, 0.2 or 0.3 wt%.

It will be appreciated that the ausferritic steel or ausferritic ductile iron may contain unavoidable impurities, although, in total, these are unlikely to exceed 0.5 wt% of the composition, preferably not more than 0.3 wt% of the composition, and more preferably not more than 0.1 wt% of the composition. The ausferritic steel alloy or ausferritic ductile iron alloy may consist essentially of the recited elements. It will therefore be appreciated that in addition to those elements that are mandatory, other non-specified elements may be present in the composition provided that the essential characteristics of the composition are not substantially affected by their presence.

The predominantly ausferritic microstructure that forms when subjecting a steel alloy or a ductile iron to a rapid austempering treatment, i.e. rapid with respect to austempering heat treatments according to the prior art, followed by baking may, if the isothermal temperature after quench and the baking temperature are different, be a mixture of coarser ausferrite with more austenite formed at higher austempering temperatures and finer ausferrite with more ferrite formed at lower austempering temperatures, i.e. temperatures closer to the initial Mₛ temperature in the austenite before quench.

However, the baking leads to a complete transformation of any remaining austenite areas of intermediate carbon content into ausferrite and equalizes the carbon distribution within the stabilized austenite phase, resulting in a more robust process providing superior and less varying mechanical properties.

The inventor has found that ausferritic steels and ausferritic ductile irons austempered in such rapid cycles followed by baking in air, for example, in an oven have several advantages over ausferritic steels and ausferritic ductile irons produced by a method according to the prior art, i.e. austempered without baking as a subsequent process step. There are namely improvements in both heat treatment performance and resulting mechanical properties of these ausferritic materials.

For example, such ausferritic steels can concurrently exhibit 0.2 % proof strengths of at least 1200 MPa, tensile strengths of at least 1700 MPa, fracture elongations of at least 14% and fracture toughness K_{JIC} of at least 150 MPa√m.

For example, such ausferritic ductile irons can concurrently exhibit 0.2 % proof strengths of at least 950 MPa, tensile strengths of at least 1300 MPa, fracture elongations of at least 6 %, and fracture toughness K_{JIC} of at least 100 MPa√m.

Due to the promotion by silicon of ferrite precipitation and growth, the time required for austempering is reduced, especially at low temperatures close above the initial Mₛ temperature. Additionally, the preferred high silicon content of 3.1-4.4 wt% Si will ensure that carbide precipitation can be avoided, not only in relatively coarse ausferrite (formed at higher austempering temperatures) with a larger amount of carbon stabilized austenite but also avoided in finer ausferrite (formed at low austempering temperatures close to initial Mₛ) with a smaller amount of carbon stabilized austenite.

Furthermore, the high silicon content also results in increased solid solution strengthening of the acicular ferrite formed, both substitutionally by silicon and interstitially by carbon (since the lattice of this ferrite is slightly tetragonal, although less so than in martensite).

The ausferritic steel and ausferritic ductile iron produced using a method according to the present invention may be further processed to make finished goods for use particularly, but not exclusively, in mining, construction, agriculture, earth moving, manufacturing industries, the railroad industry, the automobile industry, the forestry industry, metal producing, automotive, energy and marine applications, or in any other application which requires concurrently very high levels of tensile strength and ductility and/or fracture toughness and/or increased fatigue strength and/or high wear resistance, such as an application for which neither quenched and tempered martensitic nor austempered bainitic materials have sufficient properties, or in applications in which strict specifications must be met consistently.

The ausferritic steels and ausferritic ductile irons may for example be used in a suspension or powertrain-related component for use in a heavy goods vehicle or to manufacture components such as springs, spring hangers, brackets, wheel hubs, brake callipers, cams, camshafts, annular gears, clutch collars, bearings, pulleys, fastening elements, gears, gear teeth, splines, high strength steel components, load-bearing structures, armour, and/or components that must be less sensitive to hydrogen embrittlement.

### BRIEF DESCRIPTION OF THE DRAWING

The present invention will hereinafter be further explained by means of non-limiting examples with reference to the appended figure where;
- Figure 1: schematically shows the steps of a method according to an embodiment of the present invention.

### DETAILED DESCRIPTION OF EMBODIMENTS

Figure 1 shows the steps of a method for producing an ausferritic steel or ausferritic ductile iron according to an embodiment of the invention.

The method comprises the steps of: (a) heating the steel alloy or ductile iron to austenitization temperature; (b) austenitizing and, in ductile iron, saturation with carbon; (c) quenching, usually in salt bath, to avoid formation of proeutectoid ferrite or pearlite; (d) rapid but incomplete isothermal transformation to ausferrite; (e) cooling, usually to ambient temperature; (f) heating, usually in air, to continue the transformation to ausferrite; (g) baking to complete the transformation into ausferrite, equalize the carbon distribution within its austenite phase and temper any martensite previously formed; (h) cooling to ambient temperature.

### EXAMPLE

Austempered steel having the following composition in weight percent was produced using a method according to an embodiment of the present invention:

| | |
|---|---|
| C | 0.49 |
| Si | 3.30 |
| Mn | 0.87 |
| Cr | 1.19 |
| Ni | 0.59 |
| Mo | 0.14 |
| V | 0.152 |
| Cu | 0.12 |

bal. Fe and normally occurring impurities, such as 0.007 wt% P, 0.001 wt% S and 0.013 wt% Al.

A 120 tonne batch of steel having the chemical composition described above was continuously cast with 25 mm/s in six parallel strands into billets with 165x165 mm cross section and 6°m length. After vacuum annealing to remove dissolved hydrogen, four billets were preheated in a furnace at a temperature of 1200 °C for two hours, rough rolled and then rolled continuously to a final bar having 95x49 mm cross section with rounded edges (R=25 mm).

The hot rolled steel bar was fully pearlitic with Vickers hardness of 383 ±7 HV1, except for minor amounts of ≈5 % proeutectoid ferrite in the center, reducing the hardness to 359 ±18 HV1.

Six tensile testing specimens with strained diameter Ø10 mm and total length 120 mm (including Ø22 mm heads) were taken longitudinally from the hot rolled bar, austenitized at 950°C for 1 h followed by quench and isothermal transformation at 300°C for 1 h in a salt bath to form an ausferritic microstructure with hardness 492 ±5 HV30. Three of these six specimens were tested at 2 mm/minute with extensiometer distance 50 mm to determine elongation.

Tensile results were as follows: R_{p0.2}=1063 ±34 MPa; Rₘ=1783 ±16 MPa; A₅=14.8 ±1.2 %, Z=43 %.

However, the relatively low ratio R_{p0.2}/Rₘ=60 % indicated that although microstructure was completely ausferritic after 1 h at 300°C, the duration was insufficient for this highly alloyed steel to equalize its carbon distribution within the austenite phase, resulting in early plastic deformation.

To investigate if the carbon distribution in austenite could be equalized by subsequent inexpensive baking in air to complete the transformation into mechanically stable ausferrite resulting in a more robust process providing superior and less varying mechanical properties, the three remaining specimens from the austempering heat treatment were subject to a baking heat treatment in air at 250 °C for 6 h. This long baking duration at elevated temperature may not be necessary but was permitted since the high silicon content in the steel (3.30 % Si) efficiently stabilizes the already formed ausferrite by delaying/preventing any destructive transformation of its high carbon austenite films within the ausferrite into brittle bainite.

The hardness of the steel increased by baking from 492 ±5 HV30 to 506 ±7 HV30, but no changes in microstructure could be observed, since equalization of the carbon distribution within the austenite phase is invisible to optical microscopy or scanning electron microscopy, and measurements of carbon distribution in austenite films of submicron thickness would require specialized equipment.

However, tensile testing verified that the baking treatment was successful in improving the mechanical stability of the ausferritic steel.

The results were as follows: R_{p0.2}=1212 ±4 MPa; Rₘ=1710 ±2 MPa; A₅=15.6 ±0.9 %; Z=45 %.

Compared to the previous results, the 0.2 % proof strength was much higher (+14%) with an increased ratio R_{p0.2}/Rₘ=71 % being more typical for a fully transformed ausferritic microstructure. Despite the slight increase in hardness (+3 %) the ultimate tensile strength was slightly reduced (-4%) while both elongation and contraction at fracture was slightly improved. Together with the change in 0.2 % proof strength, the most remarkable improvement was the substantial reduction in scatter of measured properties, especially for 0.2 % proof strength and ultimate tensile strength, further verifying that baking contributes to a more robust process.

Austempered ductile iron having the following composition in weight percent was produced using a method according to an embodiment of the present invention:

| | |
|---|---|
| C | 3.10 |
| Si | 3.50 |
| Mn | 0.15 |
| Cu | 0.80 |
| Ni | 1.32 |
| Mo | 0.20 |
| Mg | 0.055 |

balance Fe and normally occurring impurities, such as 0.041 wt% P and 0.009 wt% S.

A 1350 kg batch of ductile iron castings weighing 29 kg each having the chemical composition described above was cast in sand molds. The Brinell hardness was in the range 245-265 HBW.

Four tensile testing specimens with Ø10 mm and total length 120 mm (including Ø22 mm heads) were taken from one casting, austenitized at 930°C for 2.5 h as recommended by the manufacturer, followed by quench in a salt bath at 330°C as recommended by the manufacturer. After 1 h, two of the specimens were taken from the salt bath and after cooling to ambient temperature baked in air at 250°C for 6 h while the remaining two were left in the salt bath for the recommended total soak time of 2.5 h. As already mentioned for the ausferritic steel, this long duration at elevated temperature may not be necessary for the ausferritic ductile iron but was permitted since the high silicon content in the ductile iron (3.50 % Si) efficiently stabilizes the already formed ausferrite by delaying/preventing any destructive transformation of its high carbon austenite films within the ausferrite into brittle bainite. In both cases the resulting microstructures were ausferritic. The specimens were thereafter tensile tested at 2 mm/minute with 50 mm extensiometer distance.
Tensile results for 330°C 2.5 h: R_{p0.2}=927 MPa; Rₘ=1202 MPa; Aₛ=2.3 %.
Tensile results for 330°C 1 h + baked 250°C 6 h: R_{p0.2}=965 MPa; Rₘ=1316 MPa; Aₛ=6.0 %.

In both cases the ratio R_{p0.2}/Rₘ was sufficiently high (74-77 %) to indicate mechanically stable ausferrite. The baking in air after much shorter soak duration in salt slightly increased both the 0.2 % proof strength and the ultimate tensile strength (+4 % vs. +9 %), while isotropic elongation at fracture (since necking is very limited in ductile irons due to its spheroidal graphite) almost tripled, from 2.3 % to 6.0 %. This is a very valuable improvement for the reliability of cast components, further verifying that baking contributes to a more robust process at considerably lower cost.

The recommendation by the manufacturer to use similar durations for the austenitization before quench and for the isothermal transformation in salt bath is due to production layout in integrated salt bath furnaces commonly used for austempering heat treatments, where one batch is austenitized in the furnace while concurrently the previous batch is isothermally transformed in the salt bath, and therefore the slower process step is determining the productivity of the plant.

The required duration for austenitization is mainly governed by temperature due to the rapid increase of carbon diffusion with increasing temperature. Higher temperature may allow for shorter duration in the furnace, while higher alloying for hardenability and larger cross sections both increases segregation of alloying elements and may thus require longer durations. Higher temperature may result in grain growth in steels, while the cast structure in ductile irons having graphite spheroids restricts grain growth. However, in contrast to tempered martensitic structures, the mechanical properties of ausferritic microstructures are not reduced by large austenite grains before quench. The main restriction for increased austenitization temperatures in integrated salt bath furnaces may be the limited creep resistance of the alloy steel structures supporting the charge, but this can be alleviated by shorter durations and reducing the furnace temperature in conjunction with change of charges in the furnace.

The required duration for the isothermal transformation in salt bath is also mainly governed by temperature but in a more complex manner, since nucleation of ferrite is stimulated by larger undercooling of the austenite at lower temperatures, while a higher transformation temperature increases the carbon diffusivity and thus improves both the growth rate of the ferrite and the increased and equalized carbon content in the carbon-stabilized austenite. Alloying for hardenability and larger cross sections both increases segregation of alloying elements and may therefore require longer durations for a complete formation of ausferrite, especially in ductile irons where transformation to ferrite is faster around the graphite spheroids and slower in intercellular areas due to enrichment of manganese, molybdenum and carbon.

Since examination of the microstructure and hardness testing alone are insufficient for determination whether the ausferrite formed is mechanically stable or not (and thus requires destructive mechanical testing), the duration recommended for isothermal transformation in the salt bath is usually suffering from larger safety margins than the duration for austenitization.

The advantages offered by this method for producing ausferritic steels and ausferritic ductile irons can be summarized as follows:
The baking is able to complete the transformation into predominantly ausferrite with high mechanical stability, on condition that carbon diffusion during the previous isothermal transformation in salt bath has sufficiently stabilized the remaining larger areas of austenite against transformation to more than minor amounts of martensite if cooled to ambient temperature, or cooled further to deliberately form martensite before baking.

The productivity in integrated salt bath furnaces can be considerably increased and the heat treatment cost substantially reduced through shortened soak time in salt bath, when combined with subsequent inexpensive baking in air in batch or belt ovens to complete the transformation into mechanically stable ausferrite, resulting in a more robust process providing superior and less varying mechanical properties. To express this in production economy terms, one may start by noting that conventional austempering in integrated salt bath furnaces is about 2-4 times more expensive than conventional austenitization, quenching in oil followed by tempering to obtain a tempered martensite structure with good toughness. Since the productivity of integrated salt bath furnaces may be doubled by running rapid austempering cycles followed by inexpensive baking, the superior mechanical properties obtained at more reasonable cost will substantially increase the applications of ausferritic steel and ausferritic ductile irons.

If martensite is formed during quench or during cooling to ambient temperature after isothermal transformation, this martensite becomes tempered during the baking in the austempering temperature range while the high silicon content prevents temper embrittlement, thus contributing to even higher strength of the predominantly ausferritic steel or predominantly ausferritic ductile iron.

Further modifications of the invention within the scope of the claims would be apparent to a skilled person. For example, it should be noted that any feature or method step, or combination of features or method steps, described with reference to a particular embodiment of the present invention may be incorporated into any other embodiment of the present invention.

## Claims

1. Method for producing an ausferritic steel or an ausferritic ductile iron, **characterized in that** it comprises the steps of subjecting a steel alloy having a silicon content of 1.5-4.4 wt% Si and a carbon content of 0.3-0.8 wt% C, or a ductile iron having a silicon content of 2.0-4.6 wt% Si and a carbon content of 2.9-3.8 wt% C, to an austempering heat treatment comprising the following steps:
- austenitizing said steel alloy or ductile iron,
- quenching said steel alloy or ductile iron at a cooling rate that is sufficiently high to prevent predominant formation of proeutectoid ferrite or pearlite,
- transforming austenite in said quenched steel alloy or quenched ductile iron into an ausferritic structure,
and subsequently
- baking said steel alloy or ductile iron at one or more temperatures to complete said transformation of any remaining austenite into ausferrite, to equalize the carbon distribution within its austenite phase, and to temper any martensite that has formed, to produce an ausferritic steel or an ausferritic ductile iron having a microstructure containing at least 50 volume-% of ausferrite.

2. Method according to claim 1, **characterized in that** said step of transforming austenite in said quenched steel alloy or said quenched ductile iron into a predominantly ausferritic structure is carried out isothermally in a salt bath.

3. Method according to claim 1 or 2, **characterized in that** said step of transforming austenite in said quenched steel alloy or said quenched ductile iron into a predominantly ausferritic structure takes place at one or more temperatures above the Mₛ temperature of the austenite, or by initially cooling said quenched steel alloy or said quenched ductile iron to form some martensite.

4. Method according to any of the preceding claims, **characterized in that** said baking step is carried out in an oven in air.

5. Method according to any of the preceding claims, **characterized in that** said ausferritic steel or said ausferritic ductile iron has a microstructure that contains less than 10 vol% of proeutectoid ferrite.

6. Method according to any of the preceding claims, **characterized in that** said ausferritic steel or said ausferritic ductile iron has a microstructure that contains less than 40 vol% of tempered martensite.

7. Method according to any of the preceding claims, **characterized in that** said method comprises the step of cooling said steel alloy or said ductile iron to ambient temperature after said austempering heat treatment and before said baking step.

8. Method according to any of claims 1-7, **characterized in that** said method comprises the step of cooling said steel alloy or said ductile iron to a temperature above ambient temperature after said austempering heat treatment and before said baking step to limit or prevent any formation of martensite.

9. Method according to any of claims 1-6, **characterized in that** said method comprises the step of cooling said steel alloy or said ductile iron to a temperature lower than ambient temperature after said austempering heat treatment and before said baking step to increase the contribution to strength from martensite tempered during said subsequent baking step.

10. Method according to any of the preceding claims, **characterized in that** said ausferritic steel or said ausferritic ductile iron has a microstructure that is substantially carbide-free or that contains less than 1 volume-% of carbides.

11. Method according to any of the preceding claims, **characterized in that** said ausferritic steel has a silicon content of 3.1-4.4 wt% Si and a carbon content of 0.4-0.6 wt% C.

12. Method according to any of the preceding claims, **characterized in that** said ausferritic steel has the following composition in weight percent:
| | |
|---|---|
| C | 0.3-0.8 |
| Si | 1.5-4.4 |
| Mn | max 4.0 |
| Cr | max 25.0 |
| Cu | max 2.0 |
| Ni | max 20.0 |
| Al | max 2.0 |
| Mo | max 6.0 |
| V | max 0.5 |
| Nb | max 0.2 |
balance Fe and normally occurring impurities.

13. Method according to any of the preceding claims, **characterized in that** said ausferritic steel exhibits at least one of the following: A 0.2% proof strength of at least 1200 MPa, a tensile strength of at least 1700 MPa, a fracture elongation of at least 14 %, and/or a fracture toughness K_{JIC} of at least 150 MPa√m.

14. Method according to any of claims 1-10, **characterized in that** said ausferritic ductile iron has the following composition in weight percent:
| | |
|---|---|
| C | 2.9-3.8 |
| Si | 2.0-4.6 |
| Mn | max 0.4 |
| Cu | max 2.0 |
| Ni | max 2.0 |
| Mo | max 0.3 |
balance Fe and normally occurring impurities.

15. Method according to any of the claims 1-10 or 14, **characterized in that** said ausferritic ductile iron exhibits at least one of the following: A 0.2% proof strength of at least 950 MPa, a tensile strength of at least 1300 MPa, a fracture elongation of at least 6 %, and/or a fracture toughness K_{JIC} of at least 100 MPa√m.
